

No. 877,171.

PATENTED JAN. 21, 1908.

F. M. F. CAZIN.

A. M. T. GAZIN.  
**METHOD OF MANUFACTURING METALLIZED ELECTRIC INCANDESCENT LAMP  
FILAMENTS.**

APPLICATION FILED AUG. 15, 1904.

4 SHEETS—SHEET 1.



## WITNESSES:

WITNESSES.  
F. C. Gibson.  
John L. Schmitt

*INVENTOR*  
*Francis M. F. Cazin.*

BY  
Fred G. Detert & Co.  
ATTORNEYS

No. 877,171.

PATENTED JAN. 21, 1908.

F. M. F. CAZIN.  
METHOD OF MANUFACTURING METALLIZED ELECTRIC INCANDESCENT LAMP  
FILAMENTS.

APPLICATION FILED AUG. 15, 1904.

4 SHEETS—SHEET 2.



Walterscoco

F. C. Gibson.  
John Schrott.

Fred G. Dietrich, Jr.  
Attorney.

Francis M. F. Cazin.

No. 877,171.

PATENTED JAN. 21, 1908.

F. M. F. CAZIN.

METHOD OF MANUFACTURING METALLIZED ELECTRIC INCANDESCENT LAMP  
FILAMENTS.

APPLICATION FILED AUG. 15, 1904.

4 SHEETS—SHEET 3.



WITNESSES:

F. C. Gibson.  
John Lechner.

INVENTOR  
Francis M. F. Cazin:

BY  
Fred G. Deternell & Co.  
ATTORNEY.

No. 877,171.

PATENTED JAN. 21, 1908.

F. M. F. CAZIN.  
METHOD OF MANUFACTURING METALLIZED ELECTRIC INCANDESCENT LAMP  
FILAMENTS.  
APPLICATION FILED AUG. 16. 1904.

4 SHEETS—SHEET 4.



# UNITED STATES PATENT OFFICE.

FRANCIS M. F. CAZIN, OF HOBOKEN, NEW JERSEY.

## METHOD OF MANUFACTURING METALLIZED ELECTRIC-INCANDESCENT-LAMP FILAMENTS.

No. 877,171.

Specification of Letters Patent.

Patented Jan. 21, 1908.

Application filed August 15, 1904. Serial No. 220,819.

*To all whom it may concern:*

Be it known that I, FRANCIS M. F. CAZIN, residing at Hoboken, in the county of Hudson and State of New Jersey, have invented 5 certain new and useful Improvements in Methods of Manufacturing Metallized Electric-Incandescent-Lamp Filaments, of which the following is a specification.

As the records of the United States Patent Office show, I had issued to me eight patents up to the date of this application, all of which relate to electric lighting and contrivances, to be used for such purpose, namely Nos. 523,460—, 523,461—, 566,285—, 620,640—, 5 621,292—, 621,292—, 640,366—, and 760,849, and that I have pending a number of applications before the U. S. Patent Office on the same line of invention and improvements, filed between February 1899 and the date of this application. All of the inventions, thus by me claimed, constitute a successive organic entirety and relate intimately to one another. I may therefore of necessity have to refer to and cite from the specifications of these my prior patents and applications, in order to fully and clearly describe my present further and new as well as useful improvements, as a further organic evolution in my persistently for long years 5 continued experimental work in the indicated line. My main purpose in such experimental work has been to substitute the carbon, used in its different physical phases as the material for electric glowers,—and thus used exclusively in the electric lamps of trade, by a better material for the purpose, viz. by metallized or metal-glowers as well as by coating these with oxids of the rare-metals. I have succeeded in this my purpose in sundry ways, described and have either disclosed these ways in my said specifications fully or in such a manner, that they became the proper object for later and special other applications, being in the first instance 5 either only vaguely alluded to, or, subject to official demand for division.

In an application of Oct. 15, 1897, on which Letters Patent No. 621,292 were issued to me on the 14th of March, 1899 I disclosed and claimed "a carbon filament, to form the negative pole in an electrolytic bath, in the shape, in which it is to be used in the lamp, without direct connection with the positive pole, such as used in the common flashing process."

Under the then prevailing rules of practice 55 I was then officially compelled to divide such disclosures and claims out of the said application. I therefore repeated such disclosures and claims in my subsequent applications, and have especially done so in my application 60 now pending No. 735,439, filed on Oct. 31, 1899, where I again disclosed and described the formation of such coating by immersing the carbon filament in a suitable electrolyte, the filament being primarily bent to shape 65 and forming the cathode of the electrolytic bath, the coating deposited being an alloy of metals of the ruthenium osmium class.

In another application filed by me on the second day of June, 1904, 210,870, I have 70 stated at length the reasons why a slight admixture of platinum is desirable in the alloy coating before referred to, and have described the coating as by preference consisting of an alloy of osmium and iridium 75 with an admixture of platinum. And in my application No. 562,189, of September 11, 1895, on which Patent No. 620,640 was granted to me on March 7, 1899, I have disclosed a new feature in the construction or making 80 of the incandescing bodies in electric lamps, namely a chemical insulation and protection as against the affinities and reactions of adjoining matter under current, be the same in a solid or in a fluid state; and in all of my 85 further disclosures of improved filaments I have reserved to myself the optional introduction or co-use of such chemical insulation and protection.

In my present application the aforesaid 90 feature as invented by me becomes of especial importance, as by its application in the form of an electrolytically deposited coating the filament becomes inert as against the affinity and reaction thereon of the oxygen 95 present in the atmosphere. With such protection or chemical insulation the vacuum-bulbs may eventually be entirely dispensed with, and when used would loose their present character as a protection of the luminescent against combustion and would remain exclusively a protection against touch or collision, that might do mechanical damage. I therefore consider my vacuum-bulbs as in no wise identical with those at present used 105 in the art of electric lighting as a protection against combustion.

It is therefore the purpose and object of

this present application for Letters Patent to primarily further protect my new and useful invention, of the above specified luminant of an electric lamp, with or without its chemical surface-protection or insulation.

It is of highest importance in a practical or commercial sense, when electric lamps, that have these described luminants are offered to the public or trade, that each individual lamp in each size or standard of light-production be virtually uniform or of equal standard with all others belonging to the same standard.

So far I have disclosed only apparatus for electrolytically plating single cores or primary carbon-filaments or at most a very limited number thereof in one and the same operation. In other words, I have mainly described and shown apparatus and methods for making samples singly of my improved filaments by means of an electrolytic process, and it is of importance, that I now also disclose method and apparatus for manufacturing those luminants on a large scale, or simultaneously under identical technical conditions, which will secure uniformity of product. To do this is the main purpose and object of this present application. I propose therefore to disclose in this application both method and apparatus for such manufacture under uniform conditions on a large and consequently economical scale, thus securing a uniform and commercially acceptable product. And I obtain such uniformity of product primarily by either of two alternate improvements in electrolytic apparatus in general or in special electrolytic apparatus for the manufacture of luminants for electric lamps. In both cases the apparatus is arranged to the effect (1) that my plural-apparatus is composed of a plurality of cells or compartments, each of which constitutes a complete single plating apparatus in itself, and that all the single apparatus in such a plural-apparatus are so arranged, that they have open connection with one another to the effect, that the same electrolyte-body can circulate through all of the single cells or compartments, each of which may contain one or more cathode-filament cores, and (2) that sundry plural-plating-apparatus are preferably interconnected for the purpose of such electrolyte circulation be it by gravity or by aid of special mechanical means, and (3) that the electric-current-conditions be uniform for all cells. It remains then for me to disclose the selective or alternate further means for obtaining the desired uniformity as between the single luminants. But it should be well understood, that each of these selective or alternate means does not only concern the uniformity as between individual luminants but concerns, and even to a higher degree, the inter-uniformity of each electrolytic coating on each single fila-

ment. The elective or alternate means for obtaining the stated uniformity consist in either one or the other of the two as herebelow stated, or in their even more preferable simultaneous application. The one consists in providing each cell with a central cathode-core and with two anode-regenerating poles and matter, which stand in line with and on opposite sides of the cathode core and on about the same level and the other (preferably used together with the two regenerating anodes but capable of use with only one anode to each cathode) consists in mechanical means for slowly revolving the cathode-core on its constructive longitudinal axis by mechanical means before one anode or between two regenerating anodes.

My improved method and apparatus for producing uniform metal deposits on cores in final filament, or luminant-shape further includes anode-troughs or cups to contain the metals required for the regeneration of the electrolyte and includes means for heating the electrolyte be it on its entire circulation or on its way locally at intervals, the latter preferably between plural apparatus, and several other contrivances and parts, their construction and arrangement, as hereinafter further described and pointed out.

For a full and clear understanding of the subject matter of this application it should be further said, that applicant has been using a great variety of chemical solutions, prepared on a great variety of formulas in the preparation of electrolytes as by him made use of in carrying out his electrolytic coating of filaments and that he has as the result of long and assiduous experimenting preferably selected some of them for his almost exclusive general use under various modifications made to adapt the filaments to the intended class, or standard functions, and that while applicant covets protection also for the by him selected formulas, he admits, that as such they all are but part and parcel of general chemical as well as physical science, as far as the components are concerned, aside of those, which are intended to form the electrolytic cathode-deposit. Applicant therefore will here further below specify the solvent conditions as by him preferably selected.

Referring to the accompanying drawings in which similar parts are designated by similar marks of reference, Figure 1, represents a single bath constructed in accordance with this invention, Fig. 2, is a plan view thereof, Fig. 3, is an end elevation of the installation of multiplex baths also in accordance with this invention, Fig. 4, is a vertical section, and Fig. 5, is a detail plan view of one of the baths shown in Fig. 3, with the cover broken away, Fig. 6, is a detail of a filament mounted in the butt preparatory to depositing thereon the metal coat, Fig. 7, is a section through a completed filament, Fig. 8, is a

plan view of an installation of Fig. 3, Fig. 9, is a detail view of the rotating cathode socket showing also the position occupied by the cathode in relation to the parts of the vat, Fig. 10, is a vertical section through a completed lamp.

Referring now to Fig. 1, the vat A is of any desired contour, for instance, elongated, and of any desired material. Thus it may be of 10 glass or of vitrified pottery. Upon the inner face of its front and rear are shelves B in which are formed cups C each of which contains a metal or metals to be applied as a coating upon the carbon filaments of the 15 lamps. A platinum wire D conducts current into each of these cups, which hold the anodes of the bath. Such a vat may be mounted in a water or oil jacket K by which it may be heated, the vat itself being carried on the 20 upper ends of pairs of pivoted levers E actuated by the screw shaft F, thus forming a pair of lazy tongs, so that upon rotating the shaft the vat may be lifted bodily from the bath and thus its temperature controlled. 25 The top G of the vat carries a suitable socket H in which the base W of one of my improved lamps may be placed to hold it while the coating is being deposited on the carbon filament b, which is secured to said base and 30 connected up in the manner pointed out in my aforesaid patent and applications, and which when the cover is in place projects within the electrolyte contained in the vat. The leading-in wires q and r of the base are 35 led through the central bore of the socket and connected to a wire D' leading to the negative pole of a suitable generator or distribution system, and thus the carbon filament forms in itself the cathode of the bath, 40 and is located at equi-distance from the anode cups, whereby as the ions travel towards it from opposite sides a uniform coating is deposited on all parts of the filament which is by preference so turned that its 45 lines are as nearly in the central plane as possible.

In large installations it is desirable to provide means for handling a number of filaments simultaneously and for this purpose the vats may be in the form of elongated 50 troughs A' which by preference are formed of wood thoroughly soaked or boiled in shellac varnish or its equivalent. These troughs are arranged in a double series of steps, with 55 passage ways M between alternate troughs as shown in Fig. 3 and 8, so that the contents of one trough may be drained in the one immediately below it, with suitable drains N' from all the troughs on each side of 60 the installation to the sumps N, from which the exhausted liquid may be led by any suitable means, such as a pump N' to the double collecting and regenerating tank O located above the installation, from the 65 opposite sides of which the hereinbefore de-

scribed cells of the troughs on the corresponding side of the steps may be fed directly by the induction pipes n' and distributing pipe n'', the latter discharging into the bottom of the several cells, while each of the 70 troughs is provided with an overflow pipe o' which are connected to the distributing pipes n'' discharging into the bottom of the several cells of the lower troughs, the overflow pipes of the lower troughs discharging directly into 75 the sump. The pipes N'—n''— and o' are all provided with suitable stop cocks by which the circulation of fluid therethrough may be controlled and directed as desired, and if desired burners n'' may be located beneath 80 the sump N and the regenerating tank O for the purpose of maintaining the electrolyte at any desired temperature, this arrangement being either additional or alternate to the arrangement of steam heating devices here- 85 inbefore described as located in the bottom of the vats themselves. Fig. 4 shows the one of the alternate arrangements, namely the one, where a series of heating pipes R passing longitudinally from end to end 90 through the trough and near to its bottom,— such arrangement necessitating the shortening below or the perforating of the glass-di- 95 vision-plates P, which is avoided in the other alternative of heating the electrolyte in the vats O. In the latter case the division-glass- 100 plates are alternately one by one reaching the bottom and not reaching the bottom to the effect, that the electrolyte is forced to flow longitudinally through the trough on its way over the top of the partition, that reaches the bottom and under the lower end of the somewhat higher partition, that does not 105 reach the bottom.

Each trough A' is supported on an insu- 110 lating base S and has on the inner faces of its front and rear a series of shelves B', each of which is provided with a depression forming the cup C', in which the metal to be deposited is contained, the length of the trough 115 being divided into a plurality of compartments by means of partitions P formed of sheet glass, inserted in the vertical groove p in the front and rear walls of the trough, the grooves being so placed that a division 120 plate is located between adjacent shelves B' on the front and rear of the vat, each trough being thus divided into a series of compartments inter-communicating at the top and bottom, each of which contains two anode 125 cups. A wire D' leading from the positive distribution wire D' of the electric circuit terminates in each anode cup, these wires being carried down into the vat through glass tubes Q into which they are sealed at the 130 lower ends, so that only the lower ends are exposed to the action of the electrolytes. These lower ends may be of platinum.

A cover G' is provided for the trough, which may be continuous from end to end 130

thereof or a series of covers may be used one for each compartment or groups of compartments, but in any event the cover or covers is provided with a socket or sockets II such as before described, a socket being located above the center of each of the compartments into which the vat is divided. By preference I hinge the covers to the rear edge of the vat by removable pintle hinges T so that a cover may be taken off with the lamp bases and filaments therein mounted and removed as a whole to the bench, upon which the bulbs are sealed onto the base, in the manner disclosed in aforesaid application. As under these conditions the covers are removed from the vats they should be made to standard and should be interchangeable one with the other.

I have said that it is a convenience to so construct the sockets II that they are adapted to receive the bases of my improved lamps to which the carbon filaments have already been secured, a base of this character with an uncoated filament attached thereto being shown in Fig. 6, and it is likewise of great importance that the filaments be each covered uniformly at all points with a selected deposit and as this can only be done by subjecting every part of the surface thereof to identical electrolytic conditions, I prefer to so mount the carbon cathode that it may be rotated in front of the anode for use with a single anode, or between oppositely placed anodes for use with a double anode hereinbefore described. To effect this the mechanism shown in Fig. 9 may be employed which consists of suitable bearing U secured to the cover G—G' of the vats, through which projects the stem h of the socket II<sup>2</sup>, the stem having a key-way h' in its upper end to which is secured a groove pulley h<sup>2</sup> around which a driving belt or cord h<sup>3</sup> passes. The stem, by preference, is hollow, through which the terminal wires q and r of the lamp pass, both of them being connected to the pulley binding post h<sup>4</sup> mounted on the upper face of the latter, a spring contact h<sup>5</sup> connected to the wire n<sup>3</sup> bearing upon the lower surface of the pulley, thus connecting the filament b of the lamp base to the negative source of current, thus making it as a whole cathode of the bath and as the pulley is rotated while current is passing all parts of such cathode the filament, will, by the rotation thereof around its longitudinal axis, be alternately moved away from and toward the anode or anodes, thus equalizing the deposit. A collar h<sup>6</sup> surrounds the stem h of the socket above the bearing, and by its adjustment, due to the set screw h<sup>7</sup>, determines the position of the socket and of the cathode when carried thereby, which adjustment, as is shown in Fig. 9, is such that the points

z between the filament b and the leading-in wires q and r are located slightly below the level of the electrolyte, although above the level of the glass partition P. Under these conditions the electrolyte deposit will also take place upon the joint, protecting the latter.

My completed lamp is shown in Fig. 16, and by preference it consists of a glass base W in which are sealed the leading-in wires q and r, and to which the filament b is secured. It is in this shape when the coat or coats is deposited upon the filament, and thereafter the base is inserted in the neck of the usual glass bulb w<sup>1</sup>, the filaments 80 properly shaped to admit this. By the aid of heat, the base W is then expanded as by blowing, or the neck of the bulb is reduced, as by spinning or both combined to cause the base to make a hermetical joint in the 85 neck of the bulb, after which the usual threaded collar w<sup>2</sup>, provided with the porcelain cap w<sup>3</sup>, and butt contact w<sup>4</sup> is fastened around the neck of the bulb, one of the leading-in wires q being secured to 90 the collar and the other to the butt contact.

The coating which I prefer to deposit upon the filament is of an alloy of metals of the ruthenium osmium class, and preferably consists of precisely the same composition, as the natural iridosmin, to the extent, that by chlorination, this mineral can be made soluble. As a rule this mineral contains a small portion of platinum. Applicant in experimenting found that 100 such presence had the effect of rendering the electrolytic metal-coating of mainly iridosmin less brittle and more ductile than a coating not containing any platinum, and applicant therefore in case of the percentage 105 of platinum present in the mineral iridosmin not being sufficient for producing the said effect to a desirable degree added chlorid of platinum to the electrolyte or in other words, platinum to the deposited alloy. It is 110 understood, that the portion of platinum thus added must be so small, that the infusibility of the other metals in the alloy be not materially lessened. The addition of a properly limited portion of platinum is 115 productive of other good qualities in the perfected filaments. It is found, that with it the deposit is smoother and of uniform texture, and is less inclined to oxidize on the surface. These qualities as stated of the 120 alloy-deposit are materially enhanced by using in the electrolyte the double-metal chlorids, where in addition to the chlorids of the named metals there are present also the chlorids of potassium, or the therewith 125 equivalent sodium-chlorids.

In a certain sense this by me preferably selected composition of my electrolyte or to more precisely state the case, of the solving agencies for the metals, which I propose to 130

electrolytically deposit, is but an analogy to the method indicated by F. Woehler as early as 1868 of absorbing osmic compounds in an alkaline fluid to form an electrolyte, from which osmium in metallic form may be precipitated. (Compare ANN/ Chem. Pharm. CXLVI--263-375.) Attention is further directed to the fact, that the regularity of the entire operation is enhanced or favored by the material contained in cups or troughs at the anode-ends of the pole-wires, which are, where not chemically insulated or protected by glass, immersed into such material, which contains the sundry metals in about the same proportion, as the desired deposit on the cores, and that these metals in these pole cups or troughs should be in the form of dust or in that of as finely divided particles as can be obtained by physical or chemical operation. It is further worth knowing, that a metal deposit, thus produced is a true alloy, the constituents of which can no longer be separated by means of the different melting temperatures of each, because the alloy has a melting temperature of its own as a whole. And this melting temperature of the alloy, as by me invented is not materially lower than that of the so-called infusible metals, but is a ductile compound-metal as against the brittleness of said metals singly. It neither should be left out of consideration, that the surface-coat of protection or chemical insulation need not of necessity be of metal, the function being performed fully and adequately if the surface-coat consists of a metal or of its oxygen compound, if the latter remains a solid coat and does not, as in the case of osmium take a gaseous form, leaving the luminant unprotected or chemically non-insulated, as all described heretofore by applicant.

It is a further feature of my present invention, that I mount the primary core on its lamp-base, or on an essential part thereof before I make use of it as the cathode in the plating cell. This has the advantage, that the completed luminant need not be further handled or manipulated except to insert and eventually seal it in one or more glass-bulbs, such a completed lamp being shown in Fig. 9.

It will be noted that not only is the bath hereinbefore described suitable for use in depositing the specific alloy but that it may be used in subsequent manipulation of the filaments and in depositing thereon such other and further coats as may be desired, as for instance, depositing upon a carbon core which has thereon the alloy coating a coating of chemical insulation to resist oxygenation, as hereinbefore suggested.

Having thus described my invention what I claim and desire to secure by Letters Patent, is:—

1. The method for producing glowers for electric incandescent lamps which consists

in coating or metallizing carbon-filaments, when bent into their final longitudinal shape, with a coat, deposit or layer or layers of metal in an electrolytic plating apparatus.

2. The method of producing glowers for electric incandescent lamps which consists in coating or metallizing carbon-filaments or graphite-filaments, when bent longitudinally into their final shape and when mounted on a base-part,—with a coat, cover, deposit or layer of metals and their alloys in an electrolytic plating apparatus.

3. The method of manufacturing glowers for electric incandescent lamps, which method consists in coating, covering including its terminals, or metallizing a filament, made of carbon or graphite, and when bent into its final longitudinal shape, and when mounted by inleading wires on a base-part, with metal in an electrolytic plating apparatus.

4. The method of manufacturing glowers for electric incandescent lamps, which method consists in coating, including terminals, filaments of carbon, that are bent into their final longitudinal shape and mounted on a base by means of inleading wires, with metal-alloy in an electrolytic plating apparatus.

5. The method of manufacturing glowers for electric incandescent lamps, which method consists in coating carbon-filaments, that are longitudinally bent into the shape intended for them in the lamp, and are mounted on a base part by means of inleading wires and terminals,—with metal in an apparatus, which consists of an interconnected series of electrolytic plating or metallizing cells.

6. The method of manufacturing glowers for electric incandescent lamps, which method consists in plating or metallizing carbon-filaments, when they are bent longitudinally into the shape intended for them as operating glowers, and when they have been mounted on a glass-base-part by means of inleading wires and their terminals, in an apparatus, which consists of a trough, divided into single electrolytic plating cells, and which cells are interconnected, to permit the circulation of the electrolyte from cell to cell, thereby securing uniformity of electrolytic deposit in quality of serial deposits, according to the electrolytes used in the apparatus.

7. The method of manufacturing glowers for electric incandescent lamps, which method consists in plating or metallizing carbon-filaments, when in their shape, intended as final, and mounted on a glass-base-part by inleading wires and terminals, with a coat of metal of the osmium-ruthenium class in electrolytic inter-connected plating cells.

8. The method of manufacturing glowers

for electric incandescent lamps, which method consists in plating or metallizing carbon-filaments, that are longitudinally bent into the shape, they are intended to have as operating glowers, and are set on a glass-base-part by means of inleading wires and terminals,—in an interconnected series of electrolytic cells with alloy (natural or artificial) of metals of the osmium-ruthenium class.

9. The method of manufacturing glowers for electric incandescent lamps, which method consists in plating or metallizing carbon-filaments, which are longitudinally bent into the shape intended for them as operating glowers, and which are set on a glass-base-part by means of inleading wires and terminals,—in an interconnected series of electrolytic cells, allowing the flow through them of the electrolyte,—with layers of metal,—the metals of highest affinity for oxygen forming the inner layer and others

following in the order as they possess less of such affinity.

10. The method of manufacturing glowers for electric incandescent lamps, which method consists in metallizing or plating graphitic filaments, which are longitudinally bent into the shape; that they are intended to have as finished glowers, and which are set on glass-base-parts by means of the in-leading wires and their terminals,—in a trough, divided into single; intercommunicating electrolytic cells, with layers of metallic alloys of different degrees of affinity for oxygen, these with the higher affinity forming the inner layers and those of the less affinity the outer layers, the outermost being allowed to oxidize on its exposed surface.

FRANCIS M. F. CAZIN.

Witnesses:

MINNA E. CAZIN,

RUDOLPH SCHROEDER.